

# UNITED STATES PATENT OFFICE.

CHRISTOPHER H. BIERBAUM, OF BUFFALO, NEW YORK.

## METHOD OF MAKING LUBRICANTS AND PRODUCTS THEREOF.

1,207,843.

Specification of Letters Patent. Patented Dec. 12, 1916.

No Drawing.

Application filed April 7, 1915. Serial No. 19,760.

To all whom it may concern:

Be it known that I, CHRISTOPHER H. BIERBAUM, a citizen of the United States, residing in the city of Buffalo, in the county of Erie, and in the State of New York, have invented new and useful Improvements in Methods of Making Lubricants and Products Thereof.

The present invention provides a method for combining petrolene with graphite and simultaneously freeing the graphite of its earthy impurities.

It is generally known by those skilled in the art, that a comparatively small amount of graphite introduced into lubricating oils and greases is highly desirable. The introduction of petrolene in proper proportions for both oils and greases is likewise very beneficial, and the object of the present invention is to provide such a lubricating product and a simple and efficient method of manufacturing the same.

The graphite is first mixed with sufficient water to make a creamy or slow flowing mass. It is then ground in a manner similar to that of mixed paints. This grinding is preferably done on the ordinary paint grinding machine suitable for that purpose and any one familiar with the operation of this class of machinery can grind the graphite to any desired degree of fineness. At this point the grading of the ground graphite by sedimentation is such that any one familiar with the art can perform this function by any of the usual methods. The most suitable grinding machines for this purpose are the bur or stone mill, either the flat or conical form.

After the graphite is ground and still in a wet condition it is then mixed with a predetermined amount of a prepared solution of petrolene, whereupon this mixture is placed in a mixing machine such as is ordinarily used in paint works, for the mixing and compounding of paints. A suitable proportion of parts for this purpose is 10 pounds of petrolene solution to 30 pounds of the wet mixture of ground graphite, this mixture consisting of substantially 14 pounds of graphite and 16 pounds of water. These ingredients are then agitated in the mechanical mixer. During the first part of the operation the mass assumes an apparently homogeneous condition, but after somewhat prolonged agitation it becomes curdy and the solid particles gradually increase in

size until finally they become one complete mass. The process very much resembles that of churning butter from cream, though the real transformation of the process is due to 60 the fact that the graphite has a greater affinity for the petrolene solution than for the water, and on the other hand the earthy impurities such as silica, iron oxid, alumina, clay and the like have a far greater affinity 65 for water than graphite has for water. For this reason the graphite is first to unite with the petrolene and the earthy materials remain in the water and so remain separated out from the pasty mass. It is essential, 70 however, that definite proportions be adhered to, as an appreciable excess of petrolene solution over and above the proportion specified does not produce the purifying effect described, while on the other hand an 75 insufficient amount of petrolene will not permit the mass to "gather."

After the process of agitation in the mechanical mixer has been continued and the water that was originally mixed with the 80 graphite and still holding the earthy materials, has been separated out from the rest of the mass, this water so eliminated should then be decanted, thereby carrying away a large part of the impurities. Thereafter, it 85 is desirable to add fresh water and continue washing since during the continuation of this process of agitation more impurities are eliminated which should be carried away by again decanting. This process of washing 90 may be prolonged to any desired degree with the result of the elimination of all undesirable impurities. As the washing and kneading processes continue, a more and more complete separation of water from the pasty 95 mass is likewise effected. By carrying this operation to a practical limit the mechanically entrained water in the graphite paste can be reduced to substantially 10%.

After the washing process is completed it 100 then becomes necessary to evaporate the final residue of water from the graphite paste. This can be done in any one of the many kinds of suitable evaporators now in general use in the various industries for just such 105 purposes. An additional amount of petrolene solution and oil should thereupon be added for further dilution. This should be done while the graphite mass is still in a heated condition and after the driving off 110 of the mechanically entrained water. For the final boiling process it is convenient to

use a mixture consisting of say 14 pounds of graphite,  $1\frac{1}{2}$  pounds of petrolene solution and 9 pounds of a light grade of mineral lubricating oil. This produces a final product which will readily mix with lubricants and at the same time give proper final proportion for use. By adding say 1% of this finished product to lubricating oil or say 2 ounces to a pound of grease the highly beneficial results of this compound can be obtained.

Petrolene is the soluble part of asphaltum and the petrolene solution before mentioned may be prepared as follows: First dissolve the asphaltum in say  $64^{\circ}$  Baumé gasolene and after that separate out the insoluble from the soluble part by filtration or sedimentation and decanting, then distil off the gasolene. It is convenient, however, to add lubricating oil before the final completion of distillation or evaporation of the gasolene by adding lubricating oil say in the proportion of 4 pounds of oil to 11 pounds of petrolene. This proportion will answer the requirements of the petrolene solution mentioned in these specifications.

The largest particle of graphite that can be carried into the oil film of a bearing is the most beneficial because it furnishes the largest quantity of graphite upon these surfaces where it is necessary when the film is squeezed out and at the same time the largest particles are the least liable to flow out from between the bearing surfaces when the oil film is destroyed. Therefore the graphite should not be ground too fine. Excessively large particles, on the other hand, have the decided drawback of settling out and also clogging the oil passages. With the strong affinity however which petrolene has for graphite very superior and satisfactory suspension of the ground graphite in lubricating oil can be effected in a manner herein disclosed.

The distinct advantages of this process are as follows: It permits grinding the graphite in water, thus producing the finest product of its kind; this also enables float-

ing the graphite in water and thus by sedimentation the ground graphite may be graded to any desired degree of fineness and uniformity. It provides for the dehydrating of the wet graphite, that is, changing the aqueous condition of the graphite into an unguent state, without first reducing the graphite to a dry state. It provides for the elimination of the earthy or mineral impurities which the graphite may contain. It furnishes the product in a convenient form in which it can be readily diluted or mixed with lubricants to any desired degree of dilution. Lastly, it provides very superior suspension of the graphite in the lubricant.

It is evident that the detailed procedure of this process and the proportions herein specified may be varied within the scope of the appended claims without departing from my invention. I, therefore do not confine myself to the exact details of operations, nor the precise proportions herein specified, but

What I do claim and desire to cover by Letters Patent is:

1. The herein described method of making a lubricant which consists in mixing a wet mass of pulverized graphite with petrolene and agitating said mixture.

2. The herein described method of making a lubricant which consists in mixing a wet mass of pulverized graphite with petrolene, agitating said mixture and diluting the mixture with oil and a solution of petrolene.

3. As a new article of manufacture, a substantially non-aqueous lubricant-mixture consisting essentially of graphite and petrolene.

4. As a new article of manufacture, a substantially non-aqueous lubricant-mixture consisting of graphite freed from impurities and petrolene.

5. As a new article of manufacture, a substantially non-aqueous lubricant-mixture consisting of graphite, petrolene and oil.

CHRISTOPHER H. BIERBAUM.

Witnesses:

W. M. DOLLAR,  
C. M. STREET.